

## UNITED STATES PATENT OFFICE

WALTER SCHROBSDORFF, OF BERLIN-WESTEND, GERMANY

## PRODUCTION OF METAL ALLOY AND OF ARTICLES MADE THEREOF

No Drawing. Application filed July 18, 1927, Serial No. 206,791, and in Germany July 21, 1926.

My invention relates to improvements in the production of metal alloys and of articles of various kinds made thereof and serving especially for such purposes as tools, implements, parts of machinery and of apparatus, nozzles, containers etc., and being used more particularly in industries and branches of manufacture, in which raw materials and partially manufactured articles are formed, shaped and otherwise worked upon under extraordinary conditions, viz., in which by reason of the physical and chemical properties of the respective materials under treatment and because of the specific conditions under which they are treated in a solid, semi-liquid or fused state said tools, implements, containers, nozzles etc. are subjected to extraordinarily high mechanical stresses and to severe attacks through high temperatures—e. g. up to 1000° centigrade—and through strong acids such as sulfuric acid, nitric acid, hot lyes etc.

The industries under consideration include those in which materials of high melting point and articles of great hardness and toughness such as chilled steel castings, articles of metal, stone, carbon, hard rubber etc. must be worked upon by turning, milling, drilling, cutting, shearing, sawing, crushing, punching, pressing, rolling, bending, drawing, die casting and other operations for which heretofore tools of refined steel, and often being provided with diamond-bits, and crucibles refractory containers nozzles etc. made of platinum were commonly used in order to meet the extraordinary requirements outlined above.

Generally stated the object of my invention is to provide new and useful metal alloys in any desired quantities for the production of what may be briefly termed hereinafter "heavy duty articles" viz, which are highly resistant against stress, heat and acids and which will comply with the extraordinary requirements under consideration to a higher degree and in a better and more comprehensive measure than it was possible heretofore with any known metal alloy both from a technical and an economical point of view.

Another object of my invention is to pro-

vide a new method by which heavy duty articles of the character set forth can be readily manufactured directly from the said metal alloys in their molten state and in such manner that the articles will require little or no finishing operations such as sharpening, 55 grinding, polishing etc.

Other objects of my invention will be dealt with hereinafter.

The nature and scope of the invention is 60 briefly outlined in the appended claims and its salient features will be more fully understood from the following specification:

According to the results of my extensive experiments metal alloys for the production 65 of articles having the aforesaid extraordinary properties can be obtained by alloying tantalum in a molten state with a metal which does not combine with carbon, i. e. which forms no carbides, such as cobalt, copper, 70 nickel, or with an element of the platinum class such as palladium, iridium, osmium viz, in such proportions that the tantalum is the quasi-solvent and predominant constituent in the particular alloy, i. e. being present in a proportion of over 50% and preferably of 88—96%.

Hitherto it has only been possible to produce mere conglomerations or mixtures of tantalum with other substances by a process 80 of sintering. Such mixtures however were not of a uniform texture, were not obtainable in a predetermined composition and consequently were unreliable in regard to their physical and chemical properties.

According to this invention genuine tantalum alloys of the aforesaid composition (as distinguished from mere mixtures) are produced in electrical high-frequency arc and resistance furnaces of types which are known 90 to metallurgical experts.

The tantalum to be alloyed may be used in its raw commercial form viz, powdered or granulated.

By this invention articles of any desired 95 shape and for any of the particular purposes concerned can be conveniently made by casting the molten tantalum alloy into carbon or graphite moulds.

Practical tests have proved that by using 100

the aforesaid metals which have no affinity for carbon as admixtures to the molten tantalum alloys are obtained which are distinguished by the properties of great active (cutting) hardness, tenacity and which will successfully withstand even high temperatures and strong acids.

In the course of my experiments tantalum has also been alloyed electrothermically i. e. in a molten state with a carbide of a metal of the chromium group viz, with a carbon compound of chromium, uranium, molybdenum, tungsten and again in such proportions that the tantalum remained the quasi-solvent predominant constituent in the alloy, being present therein in quantities of over 50% preferably of 88-96%.

Alloys of this composition which may be briefly termed for sake of convenience "carbon" tantalum alloys are distinguished from those referred to above which may be conveniently termed "non-carbon" tantalum alloys by a still greater cutting and wearing (active and passive) hardness of a diamond-like degree and will successfully withstand great heat and strong acids.

Practical tests have shown that cutting, milling, chasing, drilling tools, made by casting the molten alloy into moulds of carbon or graphite, can be successfully used for working upon articles of extraordinary hardness and toughness such as chilled steel castings, goods made of 12-14% manganese-steel etc. which hitherto have been considered as being beyond the limits of hardness within which the respective articles could be shaped and finished by steel tools, except by tools equipped with costly diamond-bits or made of vitrified abrasive substances of carborundum and the like.

In working upon materials of great hardness and toughness with tools made of tantalum alloys of the compositions hereinbefore set forth as in turning, milling and drilling, etc. the working and feeding speed and the thickness of the cut-off chips or filings can be considerably increased thereby effecting a material saving in time and production costs. E. g. material such as 12-14% manganese steel has been turned at a working speed of 180 m. per minute, the feeding speed being 7 mm. per minute and the thickness of the filings 12 mm., the corresponding figures in turning chilled steel castings being 140 m. working speed per minute, 6 mm. feeding speed per minute and 12 mm. thickness of the filings.

Other kinds of tantalum alloys have been electrothermically made in the course of my experiments which contained two additional substances as referred to above viz, one of the non-carbon group and one of the carbon group. By proportioning the amount of the admixtures to the molten tantalum solvent alloys of varying degrees of hardness and

tenacity can be obtained. Thus according to my invention alloys can be produced definitely and with any desired predetermined physical and chemical properties. E. g. tantalum alloys possessing a hardness and tenacity increased beyond that of any of its component metals can be obtained by alloying 70-98% of tantalum with 1-18% of a metal of the non-carbon group of metals and with 1-15% of a metal of the carbon-compound group hereinbefore mentioned.

All tantalum alloys produced according to my invention possess the property of resisting high temperatures of say a red heat and strong acids. Thus such alloys can be successfully used in the manufacture of drawn wire, drawn tubing etc. viz, as materials for making drawing dies for draw benches, nozzles for metal extruding presses, tools for repetition work and the like and for appliances used in industries in which strong acids are employed.

Various changes and modifications may be made in the composition of tantalum alloys specified hereinbefore and in the process of producing structural elements thereof without substantially departing from the salient features of my invention.

Since my latest experiments have shown that tantalum as the solvent and predominant element in the alloy may be wholly or partly substituted by corresponding quantities of niobium, a metal known in U. S. America as columbium which closely resembles tantalum chemically and is usually associated with the latter, I wish to expressly state that by briefly terming alloys of the compositions set forth in the foregoing specification and in the appended claims tantalum alloys I wish this term to be understood in a generic sense viz, comprising also alloys in which tantalum is replaced by the tantalum-like niobium metal or by an alloy of both said metals.

What I claim is:

1. As a new article of manufacture a cast object composed of a metal alloy containing from 50 to 98% of tantalum and a carbide of a metal of the chromium group.

2. As a new article of manufacture a cast object composed of a metal alloy containing from 50 to 98% of tantalum, 20 to 0.5% of cobalt, and a carbide of a metal of the chromium group.

3. As a new article of manufacture a cast object composed of a metal alloy containing from 50 to 98% of tantalum, 20 to 0.5% of cobalt, 10 to 0.5% of copper, and a carbide of a metal of the chromium group.

4. As a new article of manufacture a cast object composed of a metal alloy containing from 50 to 98% of tantalum, 20 to 0.5% of cobalt, 10 to 0.5% of copper, 5 to 0.5% of a metal of the platinum group including palladium, osmium, iridium, and a carbide of a metal of the chromium group.

5. As a new article of manufacture a cast object composed of a metal alloy containing from 50 to 98% of tantalum and a carbide of tungsten.

6. As a new article of manufacture a cast object composed of a metal alloy containing from 50 to 98% of tantalum, 20 to 0.5% of cobalt and a carbide of tungsten.

7. As a new article of manufacture a cast object composed of a metal alloy containing from 50 to 98% of tantalum, 20 to 0.5% of cobalt, 10 to 0.5% of copper, and a carbide of tungsten.

8. As a new article of manufacture a cast object composed of a metal alloy containing from 50 to 98% of tantalum, 20 to 0.5% of cobalt, 10 to 0.5% of copper, 5 to 0.5% of a metal of the platinum group including palladium, osmium, iridium, and a carbide of tungsten.

In testimony whereof I have signed my name to this specification.

WALTER SCHROBSDORFF.

25

30

35

40

45

50

55

60

65